

## UNITED STATES PATENT OFFICE

WALTER O. SNELLINGS, OF KINGSVILLE, TEXAS

## RAZOR-STROP DRESSING

No Drawing.

Application filed December 10, 1927. Serial No. 239,256.

This invention relates to a razor strop dressing, and the object of the invention is to provide a dressing which will preserve the strop and keep it soft and pliable for an indefinite period, which will have a fine but very effective action on the blade being stropped, and which will maintain its dressing properties as long as the strop is in serviceable condition.

10 In carrying my invention into practice I first prepare a priming composition which is suitably applied to the strop. This composition is made by dissolving 2 pounds of Venetian red, 1 pound of rosin, 2 pounds of white 15 lead and 1 pint of raw linseed oil in 1 gallon of turpentine and then adding to each quart of the mixture so prepared three quarts of varnish. This acts as a filler embodying the 20 properties of the compound which saturates the pores of the strop and provides a base coating or layer on which an intermediate coating or layer and a final coating or layer are built up.

The intermediate coating or layer is made 25 by dissolving 1 pound of Venetian red,  $\frac{1}{2}$  pound of alum,  $\frac{1}{2}$  pounds of rosin and 1 pound of white lead in 3 quarts of turpentine, and adding to each quart of the above 4 quarts of varnish. After the first or ground layer 30 has dried to a determined extent the second coating is applied in any suitable manner.

The third coating is made by dissolving  $\frac{3}{4}$  of a pound of Venetian red, 2 pounds of rosin and  $\frac{1}{2}$  pound of white lead in 2 quarts of turpentine, and then adding to each quart measure of the above 5 quarts of varnish. This is applied to the strop over the second coating and allowed to dry or harden to a certain extent, and the strop is then rubbed or smoothed 40 down by means of a smoothing or burnishing tool to remove all irregularities and to make the surface absolutely smooth, whereupon the strop is ready for use.

As stated, the first coating is used as a filler 45 for application to the raw strop, the second

coating constitutes a first surface application, and the third coating provides with the first and second coatings a dressing of the required thickness. These separate coatings are applied because a better and more uniform dressing is obtained than if the ingredients were all combined and applied as a single coating, and further as a matter of economy, as it is not necessary that the first or filler coating have the same degree of frictional properties 50 as the second and third coatings. These several coatings, of course, all blend together and make the composition homogeneous and so that the sum of their properties is obtained.

The Venetian red is used as a filler and for 55 coloring purposes, the rosin and lead blend to produce a soft abrasive compound for frictional action on the blade, the turpentine is employed as a solvent, the varnish holds the composition intact and intimately blended 60 and adds strength and durability to the strop, and the oil keeps the composition and the strop soft and pliable. The function of the alum in the intermediate coating is to act as a 65 flux or binder to assist in securing a blending 70 of the ingredients. It also has a specific action with the rosin to form a soft abrasive body, further softened by the lead, to furnish an abrasive compact to act efficiently and without harshness on the edge of the blade. 75

A dressing of this character is preferably 80 applied to canvas strops, although it may be applied to leather strops. It prevents the material of the strop from deteriorating from age and as a result of flexing actions, and it keeps the strop always soft and pliable. This dressing has a very smooth, fine and delicate action on the edge of a blade and gives a very fine, keen and smooth edge to the blade 85 which is stropped. By its use just the needed abrasive action is obtained and the edge smoothed to a high degree of keenness without wiry or other roughened surfaces liable to be produced in the use of ordinary dressings. 90

What I claim is:—

A razor strop having a dressing compound applied thereto consisting of a primary composition of Venetian red, rosin, white lead, raw linseed oil and turpentine, over which is a composition of Venetian red, alum, rosin, white lead, turpentine and varnish, and over which is a composition of Venetian red, rosin, white lead, turpentine and varnish.

10 In testimony whereof I affix my signature.  
WALTER O. SNELLINGS.

15

20

25

30

35

40

45

50

55

60

65